

## 1

2,901,336

## ANTIKNOCK COMPOSITIONS

Jerome E. Brown, Detroit, Mich., assignor to Ethyl Corporation, New York, N.Y., a corporation of Delaware

No Drawing. Application May 15, 1957

Serial No. 659,222

6 Claims. (Cl. 44—69)

This invention relates to a fundamental advance in the antiknock art. More particularly, this invention relates to gasoline compositions having markedly improved performance characteristics, notably very high octane quality and reduced engine wear tendencies.

It has long been known that lead alkyls have the highly important property of raising the octane quality of gasoline. For over 30 years, tetraethyllead has been used as the commercial antiknock agent. Over the years, improvements in refinery technology have also contributed in large measure to continuous increases in gasoline quality. In fact, the conjoint use of tetraethyllead with progressively higher octane base stocks resulting from these refinery improvements has raised the average research octane number of all premium motor fuels marketed in the United States from 86 in 1946 to 96 in 1956. By the same token, the average research octane number of all non-premium motor fuel sold in the United States went from 80 to 89 in this same period. The provision of these higher octane gasolines has, in turn, enabled the progressive development of more efficient engines. For example, the average compression ratio of passenger car engines made in this country was 50 percent higher in 1946 than it was in 1925, whereas by 1956 it was 93 percent higher than in 1925. This upward trend in engine compression ratios continues. However, a new problem has arisen in attempting to provide still higher octane quality fuels to satisfy the forthcoming higher compression engines.

To gain additional octane numbers by relying on refining methods alone has become increasingly expensive since these octane numbers are being superimposed upon fuels which already are at very high octane levels. In other words, it costs much more to refine into a fuel an incremental gain of an octane number starting with a 96 octane fuel than it does with an 86 octane fuel. Thus, the use of higher concentrations of tetraethyllead has become an economic necessity. Accordingly, the average tetraethyllead content of premium motor fuels sold in the United States has gone up from 1.5 cc. per gallon in 1946 to 2.5 cc. per gallon in 1954. In the same time period, the average tetraethyllead content of non-premium motor fuels sold in the United States has risen from 1.1 to 2.2 cc. per gallon. It is evident, therefore, that the petroleum industry is rapidly approaching the maximum permissible tetraethyllead concentration—3 cc. per gallon of motor fuel. Consequently the need exists for a new way of still further increasing fuel octane quality in an economical manner.

An object of this invention is to fulfill the foregoing need. Another object of this invention is to provide

## 2

extremely high octane quality gasolines containing a highly effective additive complement. A particular object of this invention is to provide novel gasoline compositions containing, inter alia, a minute concentration of iron pentacarbonyl which cooperates with the remainder of my novel additive complement and with the base fuel to provide especially high octane qualities. Other important objects of this invention will be apparent from the ensuing description.

10 The above and other objects of this invention are accomplished by providing gasoline having a motor octane number when clear (unleaded) of at least about 76 containing an organolead antiknock agent, preferably a tetraalkyllead compound containing from 1 to about 8 carbon atoms in each alkyl group, from about 0.4 to about 0.6 theory based on the lead of bromine as a bromine-containing scavenger, from about 0.8 to about 1.2 theory based on the lead of chlorine as a chlorine-containing scavenger, and iron pentacarbonyl, there being present in the gasoline an amount of said agent equivalent to from about 1.58 to about 3.17 grams of elemental lead per gallon and an amount of iron pentacarbonyl equivalent to from about 0.005 to 0.2 and preferably from about 0.02 to 0.1 gram of iron per gallon. These extremely small concentrations of iron pentacarbonyl—insufficient in themselves to materially raise the octane number of the unleaded base gasoline—bring about tremendous improvements in the antiknock effectiveness of the lead alkyl antiknock agent contained in the fuels of this invention. In other words, the specified amount of lead alkyl is caused by these minute concentrations of iron pentacarbonyl to exert the antiknock effectiveness that would ordinarily be exerted only by a much larger amount of lead alkyl in the absence of iron pentacarbonyl. In short, these concentrations of iron pentacarbonyl render a given quantity of lead alkyl much more effective as an antiknock than it otherwise would be. Hence, in the compositions of this invention, the iron pentacarbonyl acts as a promoter of the antiknock effectiveness of the lead alkyl.

Iron pentacarbonyl when used pursuant to this invention is also an effective inhibitor of engine wear.

As an example of the astonishing behavior of the compositions of this invention, a paraffinic fuel having a motor octane number according to ASTM Test Procedure D-357 when clear of 80 containing 3 milliliters of tetraethyllead per gallon (3.17 grams of lead per gallon), 0.5 theory of bromine as ethylene dibromide, 1.0 theory of chlorine as ethylene dichloride and only 0.05 gram of iron per gallon as iron pentacarbonyl possessed a motor performance number of 102.1 (a motor octane number of 100.7). The corresponding fuel in the absence of iron pentacarbonyl had a motor performance number of 93.3 (a motor octane number of 98.0). Thus, this minute amount of iron pentacarbonyl (0.12 cc. per gallon) in a fuel of this invention promoted the antiknock effectiveness of the tetraethyllead to such an extent that an improvement of over 8.5 performance numbers (2.7 motor octane numbers) was realized. To achieve this same gain in this fuel by the use of tetraethyllead in the absence of iron pentacarbonyl, it is necessary to use 4.6 milliliters of tetraethyllead per gallon. Therefore, this extremely small concentration of iron pentacarbonyl in a fuel of this invention made 3.0 milliliters per gallon of tetraethyllead act as if 4.6 milliliters per gallon were

present. Moreover, this enormous improvement in octane quality was achieved in a leaded gasoline composition which, in the absence of this small concentration of iron pentacarbonyl, already had a particularly high octane quality—a performance number of over 93 (a motor

each of these leaded fuels were further treated with small concentrations of iron pentacarbonyl. The various fuels were then subjected to the ASTM Research Octane Number Test—ASTM Test Procedure D-908. The results are shown in Table I.

TABLE I.—EFFECT OF FUEL ADDITIVES ON FUEL ANTIKNOCK QUALITY USING DIFFERENT OCTANE NUMBER BASE FUELS

| Cone. of $\text{Fe}(\text{CO})_5$ ,<br>g. Fe/gal. | Octane Quality Using 60 Octane<br>Base Fuel |                          |                 |                          | Octane Quality Using 80 Octane<br>Base Fuel |                          |                 |                          |
|---------------------------------------------------|---------------------------------------------|--------------------------|-----------------|--------------------------|---------------------------------------------|--------------------------|-----------------|--------------------------|
|                                                   | PN <sup>1</sup>                             | $\Delta PN$ <sup>2</sup> | ON <sup>3</sup> | $\Delta ON$ <sup>4</sup> | PN <sup>1</sup>                             | $\Delta PN$ <sup>2</sup> | ON <sup>3</sup> | $\Delta ON$ <sup>4</sup> |
| None                                              | 63.9                                        | —                        | 84.2            | —0.4                     | 85.9                                        | —                        | 95.4            | —                        |
| 0.05                                              | 63.4                                        | -0.5                     | 83.8            | -0.4                     | 87.5                                        | +1.6                     | 96.0            | +0.6                     |
| 0.1                                               | 62.8                                        | -1.1                     | 83.4            | -0.8                     | 88.9                                        | +3.0                     | 96.5            | +1.6                     |
| 0.2                                               | 62.8                                        | -1.1                     | 83.4            | -0.8                     | 89.5                                        | +3.6                     | 96.7            | +1.1                     |

<sup>1</sup> Performance number.

<sup>2</sup> Change in performance number.

<sup>3</sup> Octane number.

<sup>4</sup> Change in octane number.

octane number of 98.0). The attainment of such an improvement in this high octane region by refinery methods is extremely difficult and costly. It will also be seen that the attainment of this octane improvement could not have been accomplished in commercial practice by the sole use of additional tetraethyllead since the maximum tetraethyllead concentration currently considered permissible would have to have been exceeded by a substantial margin.

Such results are totally unexpected. It had been established heretofore that mixtures of tetraethyllead and iron pentacarbonyl were in most proportions mutually antagonistic to each other. Many mixtures of tetraethyllead and iron pentacarbonyl actually gave a lower octane number than the corresponding amount of tetraethyllead alone. Thus, in U.S. Patent 2,398,282, it was shown that in a motor fuel containing 1.32 grams of lead (1.25 cc. of tetraethyllead) per gallon, the presence of 0.21 gram of iron (0.5 cc. of iron pentacarbonyl) per gallon decreased the effectiveness of the tetraethyllead and more than 1.32 grams of lead had to be used to obtain an antiknock effect equal to that of 1.32 grams of lead alone per gallon. Furthermore, this patent shows that relatively low concentrations of iron pentacarbonyl in motor gasoline containing from less than 1 to 3.0 cc. of tetraethyllead per gallon conferred decidedly inferior antiknock qualities upon the fuel as compared with the corresponding leaded fuel not containing iron pentacarbonyl. Therefore, small amounts of iron pentacarbonyl and varying amounts of tetraethyllead were so mutually toxic that there resulted a loss of antiknock value and, therefore, the addition of iron pentacarbonyl was detrimental. In fact, it is stated in the above patent that no value was obtained from the iron pentacarbonyl until more than 0.55 gram of iron per gallon was used. This has been verified in the past by other investigators. In each instance, the addition of iron pentacarbonyl to the leaded fuel either gave the adverse effect described in the above patent or gave no benefit whatsoever. This is attributed to the fact that these prior investigators were working with entirely different gasolines (e.g., low octane fuels) and/or additive complements from those with which the present invention deals.

The unexpectedness of this invention is further shown by another series of engine tests. In these tests, two different base gasolines were used. One had a motor octane number clear of 60, whereas the other had a motor octane number clear of 80. To each of these fuels were added 3 milliliters of tetraethyllead per gallon, 0.5 theory of bromine as ethylene dibromide, and 1.0 theory of chlorine as ethylene dichloride. Portions of

25 Referring to the above data, the very small quantities of iron pentacarbonyl in the leaded fuel made from the 60 octane number base stock poisoned the tetraethyllead effectiveness so that in all cases a reduction in octane quality resulted. This directly corroborates the findings 30 described in U.S. Patent 2,398,282. However, with the fuels of this invention—made from the 80 octane number base fuel—diametrically opposite results were achieved. Thus, very large increases in antiknock quality were effected in these fuels via the promoter effect of the 35 small amounts of iron pentacarbonyl on the tetraethyllead antiknock mixture.

Another striking feature of this invention is that in the concentrations used to give the promoter effect, iron pentacarbonyl is an effective inhibitor of engine wear, 40 particularly when the engines are operated under very severe conditions. It is well known that heretofore the high engine wear caused by iron pentacarbonyl had made its use in fuel impractical. See, for example, U.S. Patents 2,546,421 and 2,546,422. Surprisingly, however, 45 substantial reductions in engine wear under drastic engine operating conditions are the direct result of the use of the extremely small concentrations of iron pentacarbonyl pursuant to this invention. This was demonstrated by a large number of engine tests.

50 Gasoline (100 motor octane number clear) containing 3 milliliters of tetraethyllead per gallon as the antiknock mixture described above was used to operate a single-cylinder engine having a displacement of 35 cubic inches at a speed of 2500 r.p.m. and a jacket temperature of

55 180° F. The intake air was filtered to prevent atmospheric dust from entering the combustion chamber. The amount of wear was determined by the method described in the December 1956 edition of Nucleonics at page 70. The criterion of engine wear was the rate 60 of loss in weight of the upper piston ring during the test period in milligrams per hour. The piston ring was a commercial chrome-plated cast iron product containing radioactive isotopes. As the surfaces of this ring were subjected to wear during engine operation, the wear 65 debris was carried into the lubricating oil where its concentration was measured by determining the radioactivity of the oil using a gamma-spectrometer. The observed count of radioactivity of the oil was directly correlated to the loss in weight of the piston ring surfaces due to wear in the operation of the engine.

70 Because of the technique employed, direct measurements were made of the chrome face wear and the iron side wear of the top piston ring. A plurality of such tests established baseline values for these two types of engine wear.

The above tests were then repeated under identical test conditions and using an identical leaded fuel to which had been added either 0.1 or 0.2 gram of iron per gallon as iron pentacarbonyl. These individual tests were carried out at the 0.1 gram of iron concentration, whereas two tests were made at the 0.2 gram concentration. The results of this series of engine tests expressed in terms of percent of baseline are shown in Table II.

TABLE II.—EFFECT OF IRON PENTACARBONYL ON ENGINE WEAR

| Iron Conc., g./gal.  | Percent of Baseline |                |
|----------------------|---------------------|----------------|
|                      | Chrome Face Wear    | Iron Side Wear |
| None (baseline)..... | 100                 | 100            |
| 0.1.....             | 60                  | 78             |
| 0.2.....             | 35                  | 58             |

As shown by the data in Table II, the fuels of this invention exhibit markedly reduced engine wear tendencies despite the expectancy based on the prior art that increased engine wear would result. The test conditions used were extremely severe and thus represent the amount of engine wear which occurs in actual service only under the most drastic operating conditions. Under milder operating conditions, the engine wear problem with conventional fuels is virtually non-existent. However, it is clear that my compositions are ideally suited for all types of engine service because under the milder operating conditions the compositions of this invention pose absolutely no engine wear problems and, as shown above, effectively reduce the wear problem under severe operating conditions. When higher concentrations of iron pentacarbonyl are used—e.g., 0.4 to 0.5 gram of iron per gallon and higher—the wear rate exceeds that of the baseline and thereby becomes excessive.

As stated above, it is preferable to use iron pentacarbonyl at concentrations from about 0.02 to 0.1 gram of iron per gallon. These concentrations take full advantage of the tremendous effectiveness of the iron pentacarbonyl as a promoter of the lead alkyl antiknock effectiveness and an inhibitor of engine wear. However, excellent results are achieved throughout the concentration range of from about 0.005 to 0.2 gram of iron per gallon as iron pentacarbonyl. At the lower end of this range, the promoter and wear inhibiting effects of iron pentacarbonyl are significant, whereas at the upper end of this range they are normally of a larger magnitude. Generally speaking, on the basis of the promoter and wear inhibiting effects and taking economic factors into consideration, the ideal concentration of iron pentacarbonyl is about 0.1 gram of iron per gallon.

To formulate the fuels of this invention, the constituents of my additive complement are blended in appropriate quantity with gasoline having a motor octane number clear of at least about 76. The order of addition of the ingredients is not critical. Thus, they can be blended separately in any order or in various sub-combinations. Because the iron pentacarbonyl concentrations are so small, it is helpful to prepare a concentrated gasoline solution containing the correct proportions of the ingredients of my additive complement and then dilute this formulation with additional gasoline to the desired concentration. Another method is to first prepare an antiknock fluid composition made up of the lead alkyl antiknock agent, the bromine-containing scavenger, the chlorine-containing scavenger, and the iron pentacarbonyl in appropriate proportions. This, in turn, is bended with the appropriate base fuel.

The following are examples of the compositions of this invention. The octane numbers of the fuels are 75

motor octane numbers clear. By definition, a theory of bromine or chlorine equals two atoms of halogen per atom of lead.

*Example I*

- 5 79.7 octane gasoline blend containing per gallon:  
 3.17 grams of lead as tetraethyllead  
 0.5 theory of bromine as ethylene dibromide  
 1.0 theory of chlorine as ethylene dichloride  
 0.05 gram of iron as iron pentacarbonyl

*Example II*

- 79.7 octane gasoline blend containing per gallon:  
 3.17 grams of lead as tetraethyllead  
 0.5 theory of bromine as ethylene dibromide  
 1.0 theory of chlorine as ethylene dichloride  
 0.1 gram of iron as iron pentacarbonyl

*Example III*

- 79.7 octane gasoline blend containing per gallon:  
 3.17 grams of lead as tetraethyllead  
 0.5 theory of bromine as ethylene dibromide  
 1.0 theory of chlorine as ethylene dichloride  
 0.2 gram of iron as iron pentacarbonyl

*Example IV*

- 25 Premium motor gasoline (81.5 octane) containing per gallon:  
 1.58 grams of lead as tetraethyllead  
 0.5 theory of bromine as ethylene dibromide  
 0.9 theory of chlorine as 1,4-dichlorobutane  
 0.1 gram of iron as iron pentacarbonyl

*Example V*

- 76 octane gasoline containing per gallon:  
 35 2.12 grams of lead as mixed methylethyllead compounds  
 0.6 theory of bromine as ethylene dibromide  
 1.0 theory of chlorine as ethylene dichloride  
 0.15 gram of iron as iron pentacarbonyl

*Example VI*

- 80 octane paraffinic gasoline containing per gallon:  
 45 3.17 grams of lead as tetraethyllead  
 0.5 theory of bromine as ethylene dibromide  
 1.0 theory of chlorine as ethylene dichloride  
 0.005 gram of iron as iron pentacarbonyl

*Example VII*

- 80 octane paraffinic gasoline containing per gallon:  
 50 3.17 grams of lead as tetraethyllead  
 0.5 theory of bromine as ethylene dibromide  
 1.0 theory of chlorine as ethylene dichloride  
 0.02 gram of iron as iron pentacarbonyl

*Example VIII*

- 55 80 octane paraffinic gasoline containing per gallon:  
 3.17 grams of lead as tetraethyllead  
 0.5 theory of bromine as ethylene dibromide  
 1.0 theory of chlorine as ethylene dichloride  
 0.1 gram of iron as iron pentacarbonyl

*Example IX*

- 80.8 octane premium fuel containing per gallon:  
 65 2.64 grams of lead as tetraethyllead  
 0.45 theory of bromine as 2,3-dibromobutane  
 1.0 theory of chlorine as ethylene dichloride  
 0.04 gram of 2,6-di-tert-butyl phenol (stabilizer)  
 0.1 gram of iron as iron pentacarbonyl

*Example X*

- 70 88 octane gasoline containing per gallon:  
 1.9 grams of lead as tetraethyllead  
 0.4 theory of bromine as dibromotoluene (mixed isomers)  
 0.8 theory of chlorine as 1,2,4-trichlorobenzene  
 0.05 grams of iron as iron pentacarbonyl

7  
*Example XI*

Isooctane (100 octane) containing per gallon:

- 3.0 grams of lead as tetraethyllead  
 0.4 theory of bromine as  $\beta,\beta'$ -dibromodiethyl ether  
 1.2 theory of chlorine as  $\beta,\beta'$ -dichlorodiethyl ether  
 0.2 gram of iron as iron pentacarbonyl

8  
*Example XII*

96 octane gasoline containing per gallon:

- 2.0 grams of lead as tetramethyllead  
 0.6 theory of bromine as acetylene tetrabromide  
 0.8 theory of chlorine as hexachlorobutadiene  
 0.03 gram of 4-methyl-2,6-di-*tert*-butyl phenol (stabilizer)  
 0.1 gram of iron as iron pentacarbonyl

9  
*Example XIII*

85.6 octane gasoline containing per gallon:

- 2.5 grams of lead as tetrabutyllead  
 0.6 theory of bromine as bromoxylenes (mixed)  
 1.2 theory of chlorine as hexachloropropylene  
 0.2 gram of iron as iron pentacarbonyl

10  
*Example XIV*

79.7 octane gasoline containing per gallon:

- 3.17 grams of lead as tetraethyllead  
 0.5 theory of bromine as ethylene dibromide  
 1.0 theory of chlorine as ethylene dichloride  
 0.03 gram of iron as iron pentacarbonyl

11  
*Example XV*

79.7 octane gasoline containing per gallon:

- 3.17 grams of lead as tetraethyllead  
 0.5 theory of bromine as ethylene dibromide  
 1.0 theory of chlorine as ethylene dichloride  
 0.06 gram of iron as iron pentacarbonyl

12  
*Example XVI*

79.7 octane gasoline containing per gallon:

- 3.17 grams of lead as tetraethyllead  
 0.5 theory of bromine as ethylene dibromide  
 1.0 theory of chlorine as ethylene dichloride  
 0.125 gram of iron as iron pentacarbonyl

Excellent antiknock qualities are exhibited by the fuels of this invention, such as those shown in the above illustrative examples. To illustrate, the fuels of Examples I through III were compared with an identical leaded fuel not containing iron pentacarbonyl using the Research Method (ASTM D-908). The results of these tests are shown in Table III.

13  
TABLE III—EFFECT OF FUEL ADDITIVES ON FUEL ANTIKNOCK QUALITY

| Example | Conc. of $\text{Fe}(\text{CO})_5$ , g. Fe/gal. | Octane Quality |      | Octane Quality Improvement Due to Promoter |                   |                      |
|---------|------------------------------------------------|----------------|------|--------------------------------------------|-------------------|----------------------|
|         |                                                | PN             | ON   | $\Delta\text{PN}$                          | $\Delta\text{ON}$ | cc. TEL <sup>1</sup> |
| I       | None                                           | 91.5           | 97.4 |                                            |                   |                      |
| I       | 0.05                                           | 94.9           | 98.5 | 3.4                                        | 1.1               | 4.3                  |
| II      | 0.1                                            | 95.6           | 98.7 | 4.1                                        | 1.3               | 4.6                  |
| III     | 0.2                                            | 95.2           | 98.6 | 3.7                                        | 1.2               | 4.4                  |

<sup>1</sup> Total amount of tetraethyllead (cc.) required in the fuel in the absence of  $\text{Fe}(\text{CO})_5$  to provide the same octane quality.

In every case the fuel of this invention had a much higher octane quality due to the presence therein of the minute amount of iron pentacarbonyl.

Similarly, the fuels of Examples VI through VIII were compared with identical fuel not containing iron pentacarbonyl using the Motor Method (ASTM D-357). The data are shown in Table IV.

14  
TABLE IV.—EFFECT OF FUEL ADDITIVES ON FUEL ANTIKNOCK QUALITY

| Example | Conc. of $\text{Fe}(\text{CO})_5$ , g. Fe/gal. | Octane Quality |       | Octane Quality Improvement Due to Promoter |                   |         |
|---------|------------------------------------------------|----------------|-------|--------------------------------------------|-------------------|---------|
|         |                                                | PN             | ON    | $\Delta\text{PN}$                          | $\Delta\text{ON}$ | cc. TEL |
| VI      | None                                           | 93.3           | 98.0  |                                            |                   |         |
| VI      | 0.005                                          | 94.2           | 98.3  | 0.9                                        | 0.3               | 3.1     |
| VII     | 0.02                                           | 97.0           | 99.1  | 3.7                                        | 1.1               | 3.6     |
| VIII    | 0.1                                            | 102.4          | 100.8 | 9.1                                        | 2.8               | 4.7     |

To further illustrate the striking octane improvements of this invention, the fuels of Examples XIV–XVI were compared with an identical fuel not containing iron pentacarbonyl using the Borderline Rating technique. The 11.3:1 compression ratio engine used in these tests was operated at 1200 r.p.m., the fuel/air ratio being 0.08 and the air and jacket temperatures being respectively  $100 \pm 5$  and  $160 \pm 5$  °F. The results are shown in Table V.

15  
TABLE V.—EFFECT OF FUEL ADDITIVES ON FUEL ANTIKNOCK QUALITY

| Example | Conc. of $\text{Fe}(\text{CO})_5$ , g. Fe/gal. | Octane Quality |       | Octane Quality Improvement Due to Promoter |                   |         |
|---------|------------------------------------------------|----------------|-------|--------------------------------------------|-------------------|---------|
|         |                                                | PN             | ON    | $\Delta\text{PN}$                          | $\Delta\text{ON}$ | cc. TEL |
| XIV     | None                                           | 100.2          | 100.1 |                                            |                   |         |
| XIV     | 0.03                                           | 103.0          | 101.0 | 2.8                                        | 0.9               | 3.3     |
| XV      | 0.06                                           | 104.0          | 101.3 | 3.8                                        | 1.2               | 4.0     |
| XVI     | 0.125                                          | 104.0          | 101.3 | 3.8                                        | 1.2               | 4.0     |

Lead alkyls which can be used in the compositions of this invention include tetramethyllead, tetraethyllead, tetrapropyllead, tetraisopropyllead, tetrabutyllead, methyltriethyllead, dimethyl-diethyllead, trimethyl-ethyllead, tetraoctyllead and the like, or mixtures thereof. Thus each alkyl group can contain from 1 to about 8 carbon atoms and be straight or branched chain. The use of tetraethyllead is preferred because of its superior performance qualities, commercial availability, and lower cost.

The bromine-containing and chlorine-containing scavengers used in the fuels of this invention are organic halide compounds which react with the lead during combustion in the engine to form volatile lead halides. It is preferable that the bromine-containing scavenger contain no chlorine and that the chlorine-containing scavenger contain no bromine, although a scavenger containing both halogens can be used, provided the scavenger mixture contains a total of bromine and chlorine within the ranges specified above. Halohydrocarbon scavengers—especially those having a vapor pressure of 0.1 to 250 millimeters of mercury at 50° F.—are preferred because of their generally superior storage stability although other scavengers can be employed successfully. Useful scavengers include ethylene dichloride, ethylene dibromide, carbon tetrachloride, propylene dibromide, 2-chloro-2,3-dibromobutane, 1,2,3-tribromopropane, hexachloropropylene, mixed bromoxylenes, 1,4-dibromobutane, 1,4-dichloropentane,  $\beta,\beta'$ -dibromodiisopropyl ether,  $\beta,\beta'$ -dichlorodiethyl ether; trichlorobenzene; dibromotoluenes; tert-butyl bromide; 2-methyl-2-bromobutane; 2,3,3-trimethyl-2-bromobutane; tert-butyl chloride; 2,3-dimethyl-2,3-dibromobutane; 2,5-dimethyl-2,5-dibromohexane; 2-methyl-2,3-dibromobutane; 2-methyl-2,3-dichlorohexane; 2,4-dibromopentane; 2,5-dichlorohexane; 3-methyl-2,4-dibromopentane; 1-phenyl-1-bromoethane; 1-phenyl-1-chloroethane; ethyl- $\alpha$ -bromoacetate; diethyl-dibromomalonate; propyl- $\alpha$ -chlorobutyrate; 1,1-dichloro-1-nitroethane; 1,1-dichloro-2-nitroethane; 1,1-dibromo-1-nitrobutane; 2-chloro-4-nitropentane; 2,4-dibromo-3-nitropentane; 1-chloro-2-hydroxyeth-

16  
17  
18  
19  
20  
21  
22  
23  
24  
25  
26  
27  
28  
29  
30  
31  
32  
33  
34  
35  
36  
37  
38  
39  
40  
41  
42  
43  
44  
45  
46  
47  
48  
49  
50  
51  
52  
53  
54  
55  
56  
57  
58  
59  
60  
61  
62  
63  
64  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
559  
560  
561  
562  
563  
564  
565  
566  
567  
568  
569  
569  
570  
571  
572  
573  
574  
575  
576  
577  
578  
579  
579  
580  
581  
582  
583  
584  
585  
586  
587  
588  
589  
589  
590  
591  
592  
593  
594  
595  
596  
597  
598  
599  
599  
600  
601  
602  
603  
604  
605  
606  
607  
608  
609  
609  
610  
611  
612  
613  
614  
615  
616  
617  
618  
619  
619  
620  
621  
622  
623  
624  
625  
626  
627  
628  
629  
629  
630  
631  
632  
633  
634  
635  
636  
637  
638  
639  
639  
640  
641  
642  
643  
644  
645  
646  
647  
648  
649  
649  
650  
651  
652  
653  
654  
655  
656  
657  
658  
659  
659  
660  
661  
662  
663  
664  
665  
666  
667  
668  
669  
669  
670  
671  
672  
673  
674  
675  
676  
677  
678  
679  
679  
680  
681  
682  
683  
684  
685  
686  
687  
688  
689  
689  
690  
691  
692  
693  
694  
695  
696  
697  
698  
699  
699  
700  
701  
702  
703  
704  
705  
706  
707  
708  
709  
709  
710  
711  
712  
713  
714  
715  
716  
717  
718  
719  
719  
720  
721  
722  
723  
724  
725  
726  
727  
728  
729  
729  
730  
731  
732  
733  
734  
735  
736  
737  
738  
739  
739  
740  
741  
742  
743  
744  
745  
746  
747  
748  
749  
749  
750  
751  
752  
753  
754  
755  
756  
757  
758  
759  
759  
760  
761  
762  
763  
764  
765  
766  
767  
768  
769  
769  
770  
771  
772  
773  
774  
775  
776  
777  
778  
779  
779  
780  
781  
782  
783  
784  
785  
786  
787  
788  
789  
789  
790  
791  
792  
793  
794  
795  
796  
797  
797  
798  
799  
799  
800  
801  
802  
803  
804  
805  
806  
807  
808  
809  
809  
810  
811  
812  
813  
814  
815  
816  
817  
818  
819  
819  
820  
821  
822  
823  
824  
825  
826  
827  
828  
829  
829  
830  
831  
832  
833  
834  
835  
836  
837  
838  
839  
839  
840  
841  
842  
843  
844  
845  
846  
847  
848  
849  
849  
850  
851  
852  
853  
854  
855  
856  
857  
858  
859  
859  
860  
861  
862  
863  
864  
865  
866  
867  
868  
869  
869  
870  
871  
872  
873  
874  
875  
876  
877  
878  
879  
879  
880  
881  
882  
883  
884  
885  
886  
887  
888  
889  
889  
890  
891  
892  
893  
894  
895  
895  
896  
897  
898  
899  
899  
900  
901  
902  
903  
904  
905  
906  
907  
908  
909  
909  
910  
911  
912  
913  
914  
915  
916  
917  
918  
919  
919  
920  
921  
922  
923  
924  
925  
926  
927  
928  
929  
929  
930  
931  
932  
933  
934  
935  
936  
937  
938  
939  
939  
940  
941  
942  
943  
944  
945  
946  
947  
948  
949  
949  
950  
951  
952  
953  
954  
955  
956  
957  
958  
959  
959  
960  
961  
962  
963  
964  
965  
966  
967  
968  
969  
969  
970  
971  
972  
973  
974  
975  
976  
977  
978  
979  
979  
980  
981  
982  
983  
984  
985  
985  
986  
987  
988  
989  
989  
990  
991  
992  
993  
993  
994  
995  
995  
996  
997  
997  
998  
999  
999  
1000  
1000  
1001  
1001  
1002  
1002  
1003  
1003  
1004  
1004  
1005  
1005  
1006  
1006  
1007  
1007  
1008  
1008  
1009  
1009  
1010  
1010  
1011  
1011  
1012  
1012  
1013  
1013  
1014  
1014  
1015  
1015  
1016  
1016  
1017  
1017  
1018  
1018  
1019  
1019  
1020  
1020  
1021  
1021  
1022  
1022  
1023  
1023  
1024  
1024  
1025  
1025  
1026  
1026  
1027  
1027  
1028  
1028  
1029  
1029  
1030  
1030  
1031  
1031  
1032  
1032  
1033  
1033  
1034  
1034  
1035  
1035  
1036  
1036  
1037  
1037  
1038  
1038  
1039  
1039  
1040  
1040  
1041  
1041  
1042  
1042  
1043  
1043  
1044  
1044  
1045  
1045  
1046  
1046  
1047  
1047  
1048  
1048  
1049  
1049  
1050  
1050  
1051  
1051  
1052  
1052  
1053  
1053  
1054  
1054  
1055  
1055  
1056  
1056  
1057  
1057  
1058  
1058  
1059  
1059  
1060  
1060  
1061  
1061  
1062  
1062  
1063  
1063  
1064  
1064  
1065  
1065  
1066  
1066  
1067  
1067  
1068  
1068  
1069  
1069  
1070  
1070  
1071  
1071  
1072  
1072  
1073  
1073  
1074  
1074  
1075  
1075  
1076  
1076  
1077  
1077  
1078  
1078  
1079  
1079  
1080  
1080  
1081  
1081  
1082  
1082  
1083  
1083  
1084  
1084  
1085  
1085  
1086  
1086  
1087  
1087  
1088  
1088  
1089  
1089  
1090  
1090  
1091  
1091  
1092  
1092  
1093  
1093  
1094  
1094  
1095  
1095  
1096  
1096  
1097  
1097  
1098  
1098  
1099  
1099  
1100  
1100  
1101  
1101  
1102  
1102  
1103  
1103  
1104  
1104  
1105  
1105  
1106  
1106  
1107  
1107  
1108  
1108  
1109  
1109<br

ane; 1-bromo-3-hydroxypropane; 1-bromo-3-hydroxybutane; 3-methyl-2-bromo-4-hydroxypentane; 3,4-dimethyl-2-bromo-4-hydroxypentane and, in general, scavengers (and lead alkyl antiknock agents) disclosed in U.S. Patents 1,592,954; 1,668,022; 2,364,921; 2,479,900; 2,479,- 902; 2,479,903; and 2,496,983.

Particularly preferred scavenger mixtures are 0.5 theory of bromine as ethylene dibromide and 1.0 theory of chlorine as ethylene dichloride; 0.6 theory of bromine as ethylene dibromide and 1.0 theory of chlorine as ethylene dichloride; and 0.45 theory of bromine as 2,3-dibromobutane and 1.0 theory of chlorine as ethylene dichloride. These mixtures effectively control the amount of deposits formed in the engine during operation and bring about this desirable result at a minimum cost.

The methods for making the above lead alkyls and scavengers, as well as iron pentacarbonyl, are well known to those skilled in the art and can be found in the literature.

Other ingredients which can be used with advantage in the fuels of this invention include dyes for identification purposes; metal deactivators, such as N,N'-di-salicylidene-1,2-diaminopropane; anti-icing and anti-rust additives; surface ignition control additives, such as tricresylphosphate, tri( $\beta$ -chloropropyl)-thionophosphate, dimethyltolylphosphate, dimethylylphosphate, trimethylphosphate, dixylylphosphoramide, trialkylphosphines, etc.; antioxidants; and the like.

The gasoline base stocks employed in this invention are preferably those which boil within or throughout the motor gasoline boiling range. This range is from about 85 to about 420° F. For best results the motor fuel should have a 90 percent boiling point of at least about 310° F. and an endpoint of at least about 375° F. These fuel base stocks are derived from a variety of refinery processes and include straight-run gasoline, catalytically or thermally cracked stocks, or gasoline hydrocarbons resulting from such processes as reforming, polymerization, isomerization, and the like. Individual gasoline hydrocarbons or various blends thereof can be used successfully. As stated above, the chief requisite of the gasoline base stock is that it have a motor octane number clear of at least 76.

I claim:

1. Gasoline having a motor octane number when clear of at least about 76 containing a lead alkyl antiknock agent, from about 0.4 to about 0.6 theory based on the

lead of bromine as a bromine-containing scavenger, from about 0.8 to about 1.2 theory based on the lead of chlorine as a chlorine-containing scavenger, and iron pentacarbonyl, there being present in the gasoline an amount of said agent equivalent to from about 1.58 to about 3.17 grams of elemental lead per gallon, and an amount of iron pentacarbonyl equivalent to from about 0.005 to 0.2 gram of iron per gallon.

2. The gasoline composition of claim 1 wherein said bromine-containing scavenger is a bromohydrocarbon and said chlorine-containing scavenger is a chlorohydrocarbon.

3. Gasoline having a motor octane number when clear of at least about 76 containing a lead alkyl antiknock agent, from about 0.4 to about 0.6 theory based on the lead of bromine as a bromine-containing scavenger, from about 0.8 to about 1.2 theory based on the lead of chlorine as a chlorine-containing scavenger, and iron pentacarbonyl, there being present in the gasoline an amount of said agent equivalent to from about 1.58 to about 3.17 grams of elemental lead per gallon, and an amount of iron pentacarbonyl equivalent to from about 0.02 to 0.1 gram of iron per gallon.

4. The gasoline composition of claim 3 wherein said bromine-containing scavenger is a bromohydrocarbon and said chlorine-containing scavenger is a chlorohydrocarbon.

5. Gasoline having a motor octane number when clear of at least about 76 containing a lead alkyl antiknock agent, about 0.5 theory based on the lead of bromine as ethylene dibromide, about 1.0 theory based on the lead of chlorine as ethylene dichloride, and iron pentacarbonyl, there being present in the gasoline an amount of said agent equivalent to from about 1.58 to about 3.17 grams of elemental lead per gallon and an amount of iron pentacarbonyl equivalent to from about 0.02 to 0.1 gram of iron per gallon.

6. The gasoline composition of claim 5 wherein said agent is tetraethyllead.

#### References Cited in the file of this patent

#### UNITED STATES PATENTS

|           |             |               |
|-----------|-------------|---------------|
| 1,666,693 | Gaus        | Apr. 17, 1928 |
| 1,903,624 | Hurley      | Apr. 11, 1933 |
| 2,398,281 | Bartholomew | Apr. 9, 1946  |
| 2,398,282 | Bartholomew | Apr. 9, 1946  |